

# UNITED STATES PATENT OFFICE.

GEORGE D. VAN ARSDALE, OF NEW YORK, N. Y.

## METHOD OF MAKING ACID AND INSOLUBLE METALLIC COMPOUNDS.

1,195,421.

Specification of Letters Patent. Patented Aug. 22, 1916.

No Drawing.

Application filed June 25, 1914. Serial No. 347,349.

To all whom it may concern:

Be it known that I, GEORGE D. VAN ARSDALE, citizen of the United States, residing at New York city, in the county of New York and State of New York, have invented certain new and useful Improvements in Methods of Making Acid and Insoluble Metallic Compounds, of which the following is a specification.

10 My present invention relates to that branch of chemistry known as hydrometallurgy and has for its primary object the provision of a method of treating metals, in solution, in such a manner that the reaction will produce, or precipitate, the dissolved metal as an insoluble, metallic salt, or compound and also produce, or form, free acid, which may later be employed in leaching out, or dissolving, more metals 20 from their ores.

More specifically, my method consists in the treatment of a solution of a salt of the metal to be precipitated, in the presence of a metal in metallic form, with a gaseous, or 25 dissolved gaseous, reducing agent, the resulting reaction precipitating the metal previously in solution and also forming free acid. This reaction is a more or less general one and produces compounds varying 30 with the metal, or metals, used and with the conditions under which the reaction takes place. But two general conditions can be noted as essential to the effectiveness of this reaction, these being, that the metal employed in the metallic state be such as to be 35 acted upon by the reducing agent used, and that the metal to be precipitated be such that its salt formed be insoluble, or at least partially insoluble, in the acid produced. 40 As will be later pointed out, these conditions, in some instances, do not interfere with the use of the same metal, in the metallic state, as that metal whose insoluble salt or compound is to be precipitated.

45 In view of the above conditions, it will be understood that hereinafter, both in the specification and claims, when I refer to a metal, as the metal to be precipitated, this reference is intended to include only such 50 metals as those which, when treated by the method described, will form salts which are insoluble or partially insoluble in the acid produced that is metals whose sulfids are

insoluble in dilute sulfuric acid. It will further be understood that when I refer to 55 a metal, as the metal to be used in metallic state, I intend to include only such metals as will be acted upon by the reducing agent employed. Also hereinafter both in the specification and claims, when I refer to a 60 reducing agent, this reference is intended to include only such reducing agents as are soluble and capable of acting upon the metal used as a precipitant.

Although other reducing agents may be 65 employed, I have found sulfur dioxid to be the most satisfactory, and this may be used either in the gaseous form or in solution.

Where sulfur dioxid is employed as the reducing agent, the results of the reaction 70 may be expressed by the following equation in which  $MSO_4$  represents a sulfate of the metal M to be precipitated and N another metal, in the metallic state:



In some cases the reaction appears to take place by the intermediate step of solution of the metallic metal N by the sulfur dioxid as 80 thio-sulfate which then reacts with the sulfate, giving as the final result, the condition represented by the above equation. In some cases, insoluble compounds, other than sulfids, may be formed. 85

It is obvious that a reaction, such as that expressed by the above formula may be made use of in a large number of ways. An example of its application is its use in the extraction of copper from ores. 90

The following formulas represent the reactions taking place upon treatment of copper sulfate solutions and copper chlorid solutions with sulfur dioxid in the presence of metallic iron: 95



These reactions may be applied in a number of ways in the hydrometallurgy of copper, some of which are given below, while others will suggest themselves to those familiar with the subject. In wet copper extraction from ores, the ores are crushed, 105

roasted if necessary and the copper afterward obtained in solution, usually by an acid solvent. There are several methods of precipitating the copper from such solutions, the most generally used heretofore, being its separation by metallic iron. In practice, however, this method has several disadvantages; among them being the fact that the cement copper produced is nearly 10 always low in copper content, due to contamination by basic iron salts, and that the liquors, from which the copper has been precipitated by iron, cannot be used again, their disposition in some cases being difficult. Furthermore in the majority of cases in which copper is extracted or separated by the employment of metallic iron, a considerable excess of iron is needed over the amount theoretically necessary for its precipitation.

By making use of the herein described reaction in precipitating copper, with iron, in the presence of sulfur dioxid, a copper precipitate may be obtained uncontaminated 25 by basic iron salts and the remaining liquors may be subsequently used for leaching additional copper ores, the formation of sulfuric acid being sufficient in some cases to render the addition of fresh acid unnecessary. The 30 amount of metallic iron needed for the complete precipitation of the copper will also, in most cases be reduced.

The best form of iron for precipitation is that kind having a large surface, such as 35 old cotton ties, tin can scrap, and the like. However, large pieces of scrap iron can be used in this method, to greater advantage than in the ordinary methods of precipitation of copper by metallic iron. This is due 40 to the fact that precipitated copper obtained by the ordinary methods is more or less adherent, therefore gathering upon the iron employed and rapidly reducing its effectiveness, making frequent cleaning necessary 45 and also necessitating the employment of long launders. On the other hand, the copper sulfid precipitate obtained by the employment of my method is not adherent and does not, therefore, reduce the efficiency of 50 the iron.

It is apparent that the method as described constitutes one step of a cycle of operations in the wet extraction of copper from its ores. Several examples of its use 55 as such a step are as follows: For example the copper from mine waters may be precipitated by this reaction. For this it is, of course, necessary to have a source of supply of sulfur dioxid gas. If the work is being 60 carried on near a smelter where roasting is done, the gases from the roasters may be used, but where such gas is not available, it may be obtained by roasting pyrites or other sulfids. If large amounts of waste gases, or

of pyrites, are available, the method may be 65 economically employed for treating comparatively dilute copper solutions. Assuming a supply of sulfur dioxid, the gas is brought into contact with the copper solution to be treated, it being of course understood that if the gas is derived directly from roasters it should be passed through some suitable dust catching apparatus before being passed into the solution. This will not only cleanse the gas, but also somewhat lower its temperature. Solution of sulfur dioxid in the copper liquor may be effected in any suitable manner, such as by the use of a tower absorbing apparatus, the construction and operation of which is well known and need not be described. The solution, after being treated with the sulfur dioxid, is then brought into contact with metallic iron, the result being the precipitation of the copper as copper sulfid and the 85 formation of free sulfuric acid in the solution. In case the precipitation of copper is not complete, heat should be applied. This may be done by utilization of waste steam or, if preferred, by blowing hot roaster 90 gases, containing, sulfur dioxid, directly into the solution without previously cooling them. Operating in this way, the reaction may take place without actual solution of the gas in appreciable quantities and the 95 first and last steps of the process united. After precipitation of the copper, the copper sulfid may be separated from the acid liquor in any one of a number of well known ways, this separation forming no 100 part of my present invention. The liquor from which the copper has been separated, will contain more or less free sulfuric acid and may, therefore, be used for dissolving copper from ores.

Another example of the use of the reaction is as a modified step of the Hunt and Douglas method. By this method cuprous chlorid is precipitated from chlorid solutions simultaneously with the regeneration 110 of free acid for leaching, by the injection of sulfur dioxid gases, while the solution is heated, or by heating the solution after the injection of such gases, the precipitated cuprous chlorid being then treated in one 115 of a number of ways to obtain metallic copper. By the Hunt and Douglas method, any silver present in the solution is not precipitated with the copper, but must be recovered from solution subsequently. In applying my reaction as a modification of the Hunt and Douglas method, metallic iron may be used either to treat the precipitated cuprous chlorid in the presence of sulfur dioxid, or by heating a solution containing 120 chlorid of copper with sulfur dioxid in the presence of metallic iron, the result in either case being the formation of insoluble cop-

per sulfid and free acid. The resulting copper precipitate is then separated from the solution by filtration or otherwise, and the remaining acid solution is then available for 5 dissolving fresh copper from its ores to provide a fresh copper solution for treatment. When this reaction is employed as a modification of the Hunt and Douglas method any silver present in the solution will be 10 precipitated or separated out with the copper.

In addition to the above examples, my method may be applied for the precipitation of copper from solutions obtained by 15 leaching ores with sulfuric acid, and in this case the resulting acid liquor is used as a part of the solvent for the fresh ores and the necessary amount of acid to be supplied thereby considerably reduced. The reaction 20 may also be used in cases where an ore is prepared for leaching by a preliminary sulfatizing roast. By precipitating the copper from solutions obtained by leaching such sulfatized ores, it is possible to regenerate 25 sufficient acid to dissolve that portion of the copper in the roasted ore, which is not soluble in water.

Other examples of possible use of the method will suggest themselves to those familiar with the subject.

Although I have as yet explained my method only in connection with the separation of copper from copper solutions, it will of course be understood that the examples thus far given are merely illustrative and that the method may be employed in separating other metals and for other purposes under varying conditions. Therefore, it will be appreciated that the equations 35 given previously, are illustrative only and may, in some cases, represent only a part of, or the final results of the reactions. I do not wish at all to limit myself to the employment of the method with any particular metal or metals and reserve the right to employ it as it may prove applicable. For example, if a solution containing sulfate of zinc, in which some sulfur dioxid has been dissolved, is heated with metallic zinc, a 40 part of the zinc is precipitated as zinc sulfid and free sulfuric acid is formed, complete precipitation being prevented by the solubility of zinc sulfid in strong acid. This reaction is represented by the following formula and serves to illustrate the fact that under some circumstances, a metal may be precipitated from its solution, by my method, by the employment of the same metal in metallic form.



Again it is possible, with my method, to

precipitate an insoluble compound of a more electro-positive metal by one less electro- 65 positive. Thus, for example, a compound of zinc may be precipitated by iron as follows:



It must be borne in mind, however, that the reaction, represented by the general formula first given, will not take place as described when the product from the salt of the metal is readily soluble in the acid produced. Thus, if a solution of ferrous sulfate containing sulfur dioxid is heated with metallic iron, no metallic compound is precipitated, since sulfid of iron is readily soluble in dilute sulfuric acid. Also aluminum 75 compounds are not precipitated as a result of the reaction. It will accordingly be apparent that the method may be used to separate metal compounds from solutions containing iron and alumina when such a result is desirable.

Having thus described the invention, what is claimed as new is:

1. The method of precipitating a metal from a solution of a salt of such metal, 90 which consists in treating the solution with sulfur dioxid and bringing the solution so treated into contact with a metal in metallic form.

2. The method of precipitating a metal 95 from a solution of one of its salts, which consists in treating the solution with sulfur dioxid and bringing the solution so treated into contact with metallic iron.

3. The method of precipitating copper 100 from a solution of one of its salts and of forming free acid, which consists in treating the copper solution with sulfur dioxid and in bringing the solution so treated into the presence of a metal in metallic form.

4. The method of precipitating copper from a solution of a salt of copper, which 105 consists in treating the solution with sulfur dioxid and bringing the solution so treated into contact with metallic iron.

5. The method of precipitating copper from a copper chlorid solution, which consists in treating the solution with sulfur dioxid and bringing the solution so treated into contact with a metal in metallic form.

6. The method of precipitating copper from a copper chlorid solution and of forming free acid, which consists in treating the solution with sulfur dioxid and bringing the solution so treated into contact with metallic iron.

7. The method of precipitating copper from a copper chlorid solution, which consists in treating the solution with sulfur dioxid in the presence of another metal in 120 metallic form.

8. The method of precipitating copper from a solution of one of its salts, which consists in treating the solution with sulfur dioxid and in bringing the solution so 5 treated into contact with another metal in metallic form.

In testimony whereof I affix my signature in presence of two witnesses.

GEORGE D. VAN ARSDALE. [L. s.]

Witnesses:

A. D. BROWN,  
F. F. BEST.